

## UNITED STATES PATENT OFFICE

2,018,660

## PRESERVATIVE PROCESS FOR CELLULOSE MATERIALS

Wallace T. Conn, Lawrence, Mass., assignor to the Government of the United States, represented by the Secretary of Commerce

No Drawing. Application October 29, 1932,  
Serial No. 640,351

5 Claims. (Cl. 91—68)

(Granted under the act of March 3, 1883, as amended April 30, 1928; 370 O. G. 757)

The invention described herein may be manufactured and used by or for the Government of the United States for governmental purposes only without the payment of any royalty thereon.

- 5 My invention relates to a preservative process for cellulose materials and particularly to one for increasing resistance to deterioration when exposed in natural bodies of water or to the atmosphere, while damp, for relatively long periods. 10 My process provides a means for increasing the resistance to deterioration of articles made of cellulose and fibrous materials such as, cotton, linen, ramie, manila, sisal, jute and other vegetable fibers, when exposed under unfavorable 15 conditions and thereby materially increasing the useful life of such articles. It is a decided improvement over preservative processes considered by my predecessor, Mr. Harden F. Taylor, in a publication entitled "Department of Commerce, 20 Bureau of Fisheries, Document No. 898."

It is a chemical treatment which will increase the present standard tensile strengths and/or resistance to deterioration.

In my co-pending application Ser. No. 624,139 I have disclosed a process for removing oily or resinous constituents which I have described as a "degumming" process, one of which comprises boiling the article for about five minutes in an aqueous solution of soap and sodium carbonate followed by a cold water rinse. A solution of one half of one per cent pure white soap and two per cent of sodium carbonate was found to give satisfactory results. In the same application I disclosed a method of mordanting in which a stock was exposed in a two per cent aqueous solution of tannic acid at one hundred and sixty degrees Fahrenheit and then in a one per cent aqueous solution of tartar emetic.

40 In the present process of treating fibrous material, I employ the same mordanting process and fixative treatment therefor, i. e., the aqueous solution of tannic acid followed by the aqueous solution of tartar emetic, as disclosed and claimed in my copending application Serial No. 624,139, 45 and set forth in the preceding paragraph, but in combination with a following treatment for the material, which comprises immersing the material, treated as above, in an aqueous solution containing potassium bichromate, of approximately 1% concentration at a temperature of approximately 200° F. for approximately 20 minutes. I have also found that the addition of copper sulphate of approximately 3% concentration and acetic acid (thirty degrees) of approximately 2% concentration to the oxidizing

bath gives additional beneficial preservative results. However, the inclusion of the latter two chemicals in the bath are not absolutely essential to accomplish satisfactory preservative results.

While the art of chrome tannage of hides and other animal products has been practiced for a long time, these methods of tanning or preservation cannot be successfully and profitably applied to vegetable products.

It is often desirable to apply to products of 10 vegetable origin, such as cotton, linen, ramie, manila, sisal, or jute, a water-proofing material such as a wax or a fat which is insoluble in water. Such water-proofing treatments do not usually conflict with the application of my method and treatments may be applied to articles 15 after receiving my chrome tanning treatment and drying, usually with better results than when applied to similar articles which have not been tanned by my method which leaves the 20 articles in a condition which permits a more thorough waxing or water-proofing.

My invention may be used for preserving fish-lines; fish nets; canvas life boat covers; life belts; awnings; sails; tents; wagon covers; tobacco cloth and other textiles used for ground coverings; sewing thread and generally to all cellulose products which are normally exposed in natural bodies of water or are exposed to the weather or to dampness.

30 The foregoing description comprehends only a general and preferred embodiment of my invention and detail changes in the process, method and compositions may be made within the scope of my claims which are therefore intended as 35 not restricted to the specific details of my invention as disclosed herein.

What I claim is:

1. A process of preserving fibrous material which comprises treating the degummed material with a mordant comprised of a heated aqueous solution of which approximately 2% is tannic acid, treating the mordanted material with a heated aqueous solution of which approximately 1% is tartar emetic, and thereafter immersing the material thus treated in an aqueous solution containing potassium bichromate of approximately 1% concentration, copper sulphate of approximately 3% concentration, and acetic acid of approximately 2% concentration at a temperature of approximately 200° F. for approximately 20 minutes.

2. A process of preserving fibrous material which comprises treating the degummed material with an aqueous solution of tannic acid,

treating the material thus treated with an aqueous solution of tartar emetic, and thereafter immersing the material thus treated in an aqueous solution containing potassium bichromate, copper sulphate, and acetic acid.

3. A process of preserving fibrous material which comprises treating the degummed material with an aqueous solution of tannic acid, treating the material thus treated with an aqueous solution of tartar emetic, and thereafter immersing the material thus treated in an aqueous solution containing potassium bichromate of approxi-

mately 1% concentration at a temperature of approximately 200° F. for approximately 20 minutes.

4. An article composed of fibrous material containing a mordant comprised of tannic acid and tartar emetic, and an oxidant preservative comprised of potassium bichromate, copper sulphate, and acetic acid.

5. An article of manufacture composed of fibrous material containing a tannic acid and tartar emetic mordant, and a potassium bichromate oxidant.

WALLACE T. CONN.